

(No Model.)

C. A. VON WELSBACK.

INCANDESCENT DEVICE.

No. 399,174.

Patented Mar. 5, 1889.



*Witnesses.*

Robert Everett,

Percy B. Hills.

*Inventor.*

Carl Auer von Welsbach.

By James L. Norvig.  
Atty.

# UNITED STATES PATENT OFFICE.

CARL AUER VON WELSBACH, OF VIENNA, AUSTRIA-HUNGARY, ASSIGNOR TO  
THE WELSBACH INCANDESCENT GAS LIGHT COMPANY, OF NEW JERSEY.

## INCANDESCENT DEVICE.

### SPECIFICATION forming part of Letters Patent No. 399,174, dated March 5, 1889.

Application filed March 8, 1887. Serial No. 230,146. (No model.) Patented in France November 4, 1885, No. 172,064; in Belgium November 4, 1885, No. 70,739; in England November 4, 1885, No. 13,342, December 12, 1885, No. 15,286, and March 13, 1886, No. 3,592; in Italy February 23, 1886, XXXVIII, 310; in Cape of Good Hope March 4, 1886, No. 6/205; in Victoria March 17, 1886, No. 4,472; in Tasmania March 24, 1886, No. 398/9; in South Australia May 3, 1886, No. 678; in New South Wales May 11, 1886, No. 1,829/2; in New Zealand June 11, 1886, No. 1,863; in Queensland June 28, 1886, No. 106; in Finland July 10, 1886, No. 261; in Spain August 10, 1886, No. 9,031/5,858; in Norway August 25, 1886, No. 88, and in India September 2, 1886, No. 40/1,145.

*To all whom it may concern:*

Be it known that I, CARL AUER VON WELSBACH, a subject of the Emperor of Austria-Hungary, residing at Vienna, in the Empire of Austria-Hungary, have invented new and useful Incandescent Devices, (for which I have obtained patents in France, dated November 4, 1885, No. 172,064; Belgium, dated November 4, 1885, No. 70,739; Italy, dated February 23, 1886, Vol. XXXVIII, No. 310; France, Certificate of Addition, dated April 22, 1886, No. 172,064; Belgium, Certificate of Addition, dated September 9, 1886, No. 74,502; Spain, dated August 10, 1886, No. 9,031/5,858; Italy, Certificate of Addition, dated October 13, 1886, Vol. XL, No. 415; Finland, dated July 10, 1886, No. 261; Norway, dated August 25, 1886, No. 88; Victoria, dated March 17, 1886, No. 4,472; New South Wales, dated May 11, 1886, No. 1,829/2; Tasmania, dated March 24, 1886, No. 398/9; Queensland, dated June 28, 1886, No. 106; New Zealand, dated June 11, 1886, No. 1,863; Cape of Good Hope, dated March 4, 1886, No. 6/205; India, dated September 2, 1886, No. 40/1,145; South Australia, dated May 3, 1886, No. 678; Great Britain, dated November 4, 1885, No. 13,342, and December 12, 1885, No. 15,286, and March 13, 1886, No. 3,592,) of which the following is a specification.

This invention has for its object to provide a novel solution for impregnating a fabric, thread, or other combustible material to manufacture incandescent devices according to the method set forth in my application filed June 8, 1886, Serial No. 204,558. In my said application I described a method of making an incandescent device by impregnating a combustible fabric or thread with aqueous or other solutions of the metallic salts of the rarer metals which produce earthy oxides, and subsequently consuming the combustible material, leaving a skeleton hood or frame composed of the earthy oxides resulting from the

decomposition of the metallic salts of the 45 metals, which, when rendered incandescent, gives out a brilliant and intense light.

The accompanying drawing illustrates a side elevation of one form of such hood or frame.

I have discovered that an excellent effect is produced by a solution of the salt of thorium alone or as an ingredient for impregnating the combustible fabric or thread, as in the following examples:

First. A solution of the salt of thorium produces a hood or frame which is rigid when rendered incandescent.

Second. A solution composed of the salts of thorium, about three parts, with two parts of magnesia, makes a hood or frame which is flexible when rendered incandescent.

Third. A solution of the salts of thorium, zirconium, and yttrium in nearly equal proportions imparts a slightly yellow tint to the 65 light.

Fourth. A solution composed of the salts of thorium, zirconium, and lanthanum in nearly equal proportions—the lanthanum a little in excess—gives a very brilliant light, 70 and the hood is flexible when rendered incandescent.

Fifth. A solution composed of one part of the salts of thorium and one part of lanthanum, with about half part of magnesia, makes 75 a hood or frame which is flexible when rendered incandescent.

Sixth. A solution of the salts of thorium, about three parts, with one of alumina, gives a hood or frame which is very flexible when 80 rendered incandescent.

In the solutions which include the salt of lanthanum for a portion of that substance the salt of yttrium may be substituted.

When a yellow light is desired, the solutions may be, seventh, a solution of the salts of thorium and lanthanum in equal proportions.

For an orange light, it may be, eighth, a solution of the salts of thorinum and neodymium in equal proportions.

For a greenish light it may be, ninth, a solution of the salts of thorinum and erbium in equal proportions.

In the mixtures 7, 8, and 9 the salt of zirconium may be substituted for a portion of the salt of thorinum. Though magnesia and alumina can be employed, as in 5 and 6, it is better to avoid the use of much of these substances, as incandescent devices containing them are not so durable.

For impregnating the fabric or thread, an aqueous or other solution of the salt of thorinum is employed alone or in connection with another salt of the metal or metals, as set forth.

In preparing the solution I prefer to use the nitrate of the metal, as it is generally soluble; so, also, but in less degree, iodide or bromide of the metal.

The solution containing the salt having been prepared, the fabric or thread is im-

pregnated therewith, and then the impregnated fabric or thread is subsequently exposed to the heat of a flame, whereby the fabric or thread is consumed, leaving a skeleton hood or frame composed of the product of the decomposed salt or salts, which is thorium oxide alone or in connection with the other ingredients mentioned.

Having thus described my invention, what I claim is—

1. An incandescent composed of the oxide of thorinum, substantially as described.

2. A filament, fabric, or textile frame of combustible material impregnated with a salt of thorinum in aqueous solution, substantially as set forth.

In testimony whereof I have signed my name to this specification, in the presence of two subscribing witnesses, this 24th day of May, A. D. 1886.

CARL AUER VON WELSBACH.

Witnesses:

VICTOR TISCHLER,  
EDMUND JUSSEN.